

## UNITED STATES PATENT OFFICE

2,665,205

## HOT WORK STEEL ALLOY

Leonard V. Klaybor, Dunkirk, N. Y., assignor to  
Allegheny Ludlum Steel Corporation, Bracken-  
ridge, Pa., a corporation of Pennsylvania.

No Drawing. Application October 13, 1951,  
Serial No. 251,243.

6 Claims. (Cl. 75—126)

1

This invention relates to an improved hot work alloy steel and particularly, to a hot work alloy having a high abrasion resistance and a good impact strength.

A hot work alloy having wide usage in dies, etc., used in hot forging, hot pressing and hot extrusion of steels, aluminum, copper, brass and any metal normally worked at elevated temperatures. Heretofore, it has been customary to employ a 5% chromium steel having a low maximum carbon content of under .60%, usually well under .50% (.30 to .40%) for such an application. It has been necessary to maintain a lower carbon content to provide it with increased toughness and to increase the high temperature fatigue failure of its working surface (phenomenon commonly referred to as heat checking). However, such an alloy has a relatively poor abrasion resistance and for this reason, has not been entirely satisfactory.

In endeavoring to solve the problem thus presented, I determined that it must be done in such a manner as to not adversely alter other required physical properties or adversely affect the heat treatment of the alloys. I discovered that the problem could be solved by increasing the carbon content above the maximum previously permissible amount and adding titanium as an alloying element, both within critical and essential ranges.

It thus has been an object of my invention to provide a practical solution to the problem.

Another object has been to develop a relatively inexpensive hot work alloy steel that will have a greatly increased abrasion resistance without a sacrifice of a good impact strength, toughness, heat checking and other required properties.

A further object has been to provide a titanium containing hot work steel alloy suitable for heat treatment and for use in hot dies.

In carrying out my invention, I discovered that the advantages of a lower carbon content could be retained by employing titanium in proper amounts as an alloying and carbide forming element and that a resulting, greatly increased abrasion resistance with a good impact strength could be obtained in the alloy without adversely

2

affecting its other properties. The alloys of my invention have the following contents:

TABLE I

|                                            | Optimum       |
|--------------------------------------------|---------------|
| C=0.60 to 1.25%                            | 0.85 to 0.95% |
| Cr=3.00 to 6.00%                           | 5.00 to 5.50% |
| Ti=2.00 to 3.50%                           | 3.00 to 3.25% |
| Si=0.10 to 1.50%                           | 0.90 to 1.10% |
| Mo=0.50 to 2.00%                           | 1.10 to 1.30% |
| W=0.50 to 2.00%                            | 1.10 to 1.40% |
| Mn=up to 0.50%                             | 0.30 to 0.50% |
| V=up to 1.00%                              | 0.50% maximum |
| Remainder iron with incidental impurities. |               |

In these alloys, heat treatment and impact strength do not deviate from the standard 5% chromium, titanium-free, 35% carbon hot work steel alloy. A measure of the increased hot abrasion resistance was obtained by subjecting samples of my alloys to the action of a rotating disc of a super high temperature alloy at 1700° F. under a pressure of 40 pounds. The heated disc was rotated through a distance of 120,000 feet peripheral wheel travel at a speed of 100 R. P. M. against the alloy samples. The weight loss of the test samples A of my alloy were recorded. Comparison alloy steels B and C were also subjected to the same test, see Table II.

TABLE II  
CONTENT

| Steel | C       | Cr      | Ti      | Si      | Mo      | W       | Mn      | V       |
|-------|---------|---------|---------|---------|---------|---------|---------|---------|
|       | Percent | Percent | Percent | Percent | Percent | Percent | Percent | Percent |
| A     | 0.86    | 5.74    | 3.06    | 1.20    | 1.60    | 1.17    | 0.49    | —       |
| B     | .35     | 5.61    | —       | 1.05    | 1.34    | 1.26    | .34     | 0.23    |
| C     | .41     | 4.11    | —       | .36     | —       | 9.22    | .41     | .48     |

## WEIGHT LOSS AFTER HOT ABRASION TEST

| Steel | Hardness<br>Rockwell<br>C | Weight loss<br>(grams X<br>10) |
|-------|---------------------------|--------------------------------|
| A     | 48                        | 0.56                           |
| B     | 47                        | 1.17                           |
| C     | 51.5                      | 1.35                           |

45 The data of Table II clearly show the marked improved effect of titanium and additional carbon. That is, these two critical elements in properly proportionate ranges give the alloy a hardness and abrasion resistance under conditions of hot usage and as illustrated by Table III, without

adversely affecting other requisite physicals. I have determined that as a minimum, the carbon content should be increased by .15 to .25% for each 1% additional titanium starting with .60% carbon and 2% titanium.

In Table III, specimens used were 1 inch round by 2 inches long and were oil quenched from the indicated temperatures. All were tempered for two hours at the indicated temperatures.

TABLE III

## Analysis

Alloy A (mine), see Table II.

Alloy D (comparison):

C=.38%, Cr=5.04%, Si=1.00%, Mo=1.87%.  
W=1.60%, Mn=.38%, and V=.20%.

## ALLOY A

| Hardening temp., ° F. | As quenched hardness Rc | Sheppard fracture rating | Hardness Rk C after tempering 2 hrs. at— |           |           |           |
|-----------------------|-------------------------|--------------------------|------------------------------------------|-----------|-----------|-----------|
|                       |                         |                          | 900° F.                                  | 1,000° F. | 1,100° F. | 1,200° F. |
| 1,800                 | 50.5                    | 7                        | 51.5                                     | 51        | 44        | 36        |
| 1,850                 | 52                      | 7                        | 52.5                                     | 53        | 46        | 37        |
| 1,900                 | 53                      | 8                        | 53.5                                     | 54        | 47        | 38        |
| 1,950                 | 54                      | 8                        | 54                                       | 55        | 48        | 39        |

## ALLOY D

|       |      |    |      |      |      |    |
|-------|------|----|------|------|------|----|
| 1,800 | 51   | 8  | 51.5 | 53   | 51.5 | 40 |
| 1,850 | 53   | 8½ | 53   | 54.5 | 52   | 42 |
| 1,900 | 54.5 | 9  | 54   | 55   | 53   | 43 |
| 1,950 | 56   | 9  | 55   | 56   | 53   | 43 |

The titanium bearing alloy A is slightly lower in hardness because it is on the low side of the carbon content for the titanium content involved. A .95% carbon containing alloy of my invention produces more nearly equal results to alloy D.

## What I claim is:

1. An improved hot work die type of steel alloy which is tempered by heat treatment which contains about .60 to 1.25% carbon, about 3 to 6% chromium, about 2 to 3.5% titanium, about .10 to 1.5% silicon, about .50 to 2% each of molybdenum and tungsten, up to about .50% manganese, up to about 1% vanadium, and the remainder iron with incidental impurities; the carbon

and titanium being highly essential in the ranges set forth, and the alloy being characterized by its high hot abrasion resistance with a good impact strength.

5 2. An alloy as defined in claim 1, wherein the maximum vanadium content is about .50%.

3. An alloy as defined in claim 1, wherein starting from the minimum specified amounts of carbon and titanium, the carbon is increased by at least .15 to .25% for each 1% increase in amount of titanium.

10 4. An alloy as defined in claim 1 wherein, its above defined abrasion resistance is retained after it has been tempered for about two hours at a temperature within a range of 900° F. to 1200° F.

15 5. An improved hot work die type of steel alloy which is tempered by heat treatment which contains about .85 to .95% carbon, about 5 to 5.5% chromium, about 3 to 3.25% titanium, about .90 to 1.10% silicon, about 1.10 to 1.30% molybdenum, about 1.10 to 1.40% tungsten, about .30 to .50% manganese, about .50% maximum vanadium, and the remainder iron with incidental impurities; the alloy being characterized by its high hot abrasion resistance with good impact strength in its tempered condition.

20 6. An improved hot work die type of steel alloy having a high hot abrasion resistance combined with a good impact strength whose alloying ingredients consist essentially of about .60 to 1.25% carbon, about 3 to 6% chromium, about 2 to 3.5% titanium, about .10 to 1.5% silicon, about .50 to 2% each of molybdenum and tungsten, up to about .50% manganese, up to about 1% vanadium, and in which the carbon is increased by .15 to .25% for each 1% additional titanium within the stated ranges of each, starting with .60% carbon and 2% titanium.

25 LEONARD V. KLAYBOR.

## References Cited in the file of this patent

## UNITED STATES PATENTS

45 Number Name Date  
2,343,069 Luerssen et al. Feb. 29, 1944